

Patented Oct. 6, 1931

1,826,656

# UNITED STATES PATENT OFFICE

ADOLF FRY, OF ESSEN, GERMANY, ASSIGNOR, BY MESNE ASSIGNMENTS, TO THE  
NITRALLOY CORPORATION, A CORPORATION OF DELAWARE

## PROCESS FOR EXTERNALLY HARDENING CAST IRON AND ARTICLE OF MANUFACTURE PRODUCED THEREBY

No Drawing. Application filed January 30, 1928, Serial No. 250,729, and in Germany March 17, 1927.

The invention has for its object a process for hardening the marginal layers of cast iron, which process is carried out without any quenching operation and by which a cast iron 5 is produced that is hard on its surface and possesses a particularly high resistance to wear. This object is attained according to the invention by subjecting a suitably alloyed cast iron (alloyed e. g. with aluminium) at 10 comparatively low temperatures and for a sufficiently long time to the action of substances which give off nitrogen.

The process may be carried out for instance in the following manner: Cast iron articles 15 are manufactured by casting into sand moulds, of a cast iron alloyed with about 1 per cent of aluminium. These aluminium-containing cast articles after they have become cold may be brought into the desired finished 20 shape by suitably machining them by means of cutting tools with the ease and in a similar manner as gray cast iron. After being machined, the cast articles are put into a closed receptacle to which a gas is supplied that will liberate nitrogen, the receptacle having an 25 outlet for the non-absorbed portions of the gas supplied. In this receptacle the articles are exposed at a temperature of about 500 degrees C. and for a sufficiently long time 30 (more than 24 hours) to the action of gases containing, and capable of setting free, nitrogen. At this temperature the nitrogen penetrates into the cast articles, and according 35 to the duration of the action of the nitrogen upon the cast articles, a more or less high degree of hardness of the surface of the articles is obtained. After the action of the nitrogen, the cast articles are slowly cooled 40 without quenching them. In this manner the surfaces of the articles may have imparted to them in a simple way hardnesses of about 650 to around 750-800 on the Vickers-Brinell hardness scale. These degrees of hardness 45 approximately correspond to the Vickers-Brinell hardnesses of hard chill castings and secure a very high resistance to wear.

Besides aluminium, other elements that produce a definite improvement in the ability to acquire hardness by introduction of nitrogen when brought into contact therewith may

be used as alloying additions. Examples of elements that may be so used are silicon, manganese, chromium, nickel, cobalt, vanadium, molybdenum, tungsten, titanium, zirconium and the like, either separately or in any desired combination. It will be understood 55 that the proportions of these various elements that should be added to produce the desired nitriding effect will vary somewhat, depending upon the alloying element or elements used and further depending upon the results desired, such as for example whether a thick case is desired or a relatively thin case with higher surface hardness. Consideration may also be given to the known properties of certain of the elements to effect structural improvement in the alloy being nitrided. In the case of the elements silicon and manganese, which are generally present in some amount in cast iron, it will be understood 60 that the proportions of these must be increased to what in effect are alloying proportions as distinguished from normal proportions if reliance is to be had on these elements or either of these elements alone for promoting the nitriding effect.

The addition of aluminium, chromium, etc. to relatively low carbon steels and steel alloys, i. e., steels containing up to about 0.6% carbon, to improve their nitride hardening properties was disclosed in my earlier patents Nos. 1,487,554 and 1,649,398. However, when similar additions were made to such steels and steel alloys containing greater amounts of carbon it was found that the increased hardness due to the nitriding effect decreased with increasing carbon content, so much so as to indicate very clearly that if the nitriding treatment were to be applied to a ferrous alloy containing a carbon content 80 characteristic of cast iron, no substantial increase in hardness would result. Consequently, it is surprising to find that when the carbon range characteristic of cast iron is 85 reached, the addition of aluminium, or any one of the other alloying elements specified, either alone or in any desired combination, is effective to bring about a definite improvement in the nitriding properties.

When in the following claims aluminium 100

alone is indicated as an alloying constituent, all substances are to be understood thereby, as for instance the above indicated ones, which produce the effect hereinbefore indicated.

It is to be understood that wherever in the claims the term "compound" is used in referring to the hardened layer such term is not limited to a definite chemical compound but 10 may comprise a mixture of various chemical compounds, e. g., nitrides, which may be binary, ternary or more complex, and will ordinarily be present principally in the form of a solid solution.

15 What I claim and desire to secure by Letters Patent, is:—

1. The process comprising subjecting cast iron containing about 1 per cent of aluminium at a temperature of about 500 degrees C. to 20 the action of a nitrogen-liberating substance.

2. The process comprising subjecting cast iron containing about 1 per cent of aluminium at a temperature of about 500 degrees C. more than 24 hours to the action of a 25 nitrogen-liberating substance.

3. The process comprising subjecting cast iron containing about 1 per cent of aluminium at a temperature of about 500 degrees C. more than 24 hours to the action of a nitrogen- 30 liberating gas.

4. The process comprising subjecting cast iron containing about 1 per cent of aluminium and an addition of at least one of the elements comprising the group: silicon, manganese, chromium, nickel, cobalt, vanadium, 35 molybdenum, tungsten, titanium, zirconium, at a temperature of about 500° C., to the action of a nitrogen-liberating substance.

5. The process, comprising subjecting cast 40 iron containing about 1 per cent of aluminium and an addition of more than one of the elements selected from the group comprising: silicon, manganese, chromium, nickel, cobalt, vanadium, molybdenum, tung- 45 sten, titanium, zirconium, at a temperature of about 500° C. to the action of a nitrogen-liberating substance.

6. The process comprising subjecting cast iron, containing about 1 per cent of aluminium and an addition of a substance adapted to 50 improve the strength of the cast iron, to the action of a nitrogen-liberating gas at a temperature of about 500 degrees C. more than 24 hours.

55 7. The process comprising subjecting cast iron, containing about 1 per cent of aluminium and another substance adapted to improve the capacity of being hardened by nitriding, of the cast iron, to the action of a 60 nitrogen-liberating gas at a temperature of about 500 degrees C. more than 24 hours.

8. An article hardened in its marginal layer by nitriding, and consisting of a cast iron alloy containing about 1 per cent of aluminium.

9. An article hardened in its marginal layer by nitriding, consisting of a cast iron alloy containing about 1 per cent of aluminium, and as a further alloying addition at least one of the elements selected from the 70 group: silicon, manganese, chromium, nickel, cobalt, vanadium, molybdenum, tungsten, titanium, zirconium.

10. An article hardened in its marginal layer by nitriding, consisting of a cast iron 75 alloy containing about 1 per cent of aluminium, and as further alloying conditions a combination of elements selected from the group: silicon, manganese, chromium, nickel, cobalt, vanadium, molybdenum, tungsten, 80 titanium, zirconium.

11. An article hardened in its marginal layer by nitriding and consisting of a cast iron containing an alloying addition having substantially the same properties as aluminium as regards ability to form with iron and nitrogen a hard compound when nitrided, said addition being present in small but effective proportions.

12. An article hardened in its marginal layer by nitriding and consisting of a cast iron containing an effective and substantial proportion of an alloying addition, such as one or more of the elements aluminium, silicon, manganese, chromium, nickel, cobalt, 95 vanadium, molybdenum, tungsten, titanium, zirconium, having the property of promoting the formation of a hard and adherent nitrided layer when such article is subjected to a nitriding treatment.

The foregoing specification signed at Cologne, Germany, this 13th day of January, 1928.

ADOLF FRY.

105

110

115

120

125

130

**CERTIFICATE OF CORRECTION.**

Patent No. 1,826,656.

Granted October 6, 1931, to

**ADOLF FRY.**

It is hereby certified that error appears in the printed specification of the above numbered patent requiring correction as follows: Page 2, line 18, claim 1, for "aluminum" read aluminium; line 35, claim 4, for "nickle" read nickel, and line 77, claim 10, for "conditions" read additions; and that the said Letters Patent should be read with these corrections therein that the same may conform to the record of the case in the Patent Office.

Signed and sealed this 8th day of December, A. D. 1931.

**M. J. Moore,**  
Acting Commissioner of Patents.

(Seal)